

## UNITED STATES PATENT OFFICE

2,370,268

## PAPER-COATING COMPOSITION

Charles W. Stewart, River Forest, Ill., assignor to  
 Corn Products Refining Company, New York,  
 N. Y., a corporation of New Jersey

No Drawing. Original application October 1,  
 1941, Serial No. 413,128. Divided and this ap-  
 plication September 13, 1943, Serial No. 502,198

## 1 Claim. (Cl. 106—150)

This invention relates to the coating or filling of paper or like material with china clay, precipitated chalk, precipitated barium sulfate (blanc fixe), talc, titanium pigment, or other inert, argillaceous or mineral substance used for closing the pores of the paper so as to give the paper a glossy surface and make it suitable, for example, for printing. The term "inert filling material," as used herein, is intended to include any and all materials used for this purpose; and when the term "clay" is used in the description, it will be understood that in place of clay any other suitable inert filling material may be employed as an equivalent.

This application is a division of application Serial No. 413,128, filed October 1, 1941.

It has been customary heretofore to use casein as an adhesive or binder for the clay in compounds of this type; the coating consisting in such case, essentially, of clay, or other inert filling material, casein dissolved by an alkali or alkaline salt such as borax or soda ash, and water. The compound is ordinarily applied to the paper either by a roll coating machine or by a brush coating machine, after which the coated paper web is tightly drawn over a moving rubber apron or revolving drum. It is then dried in suitable drying apparatus, for example, in a festoon drier, through which the paper webs, hung in loops from supports are moved in an atmosphere controlled as to temperature and humidity. Finally, the coated paper is subjected to pressure between weighted calender rolls.

The present invention is based upon the discovery that it is possible, and moreover practically feasible, to substitute for casein in paper coating compounds zein, the alcohol soluble constituent of corn (maize) protein, provided the zein be dissolved or dispersed by the use of suitable dispersing agents as hereinafter described; and further, that by this substitution several very important and unexpected advantages are obtained namely:

(1) The preparation and mixing of the ingredients is simplified and made less costly. The zein-clay compound can be produced by merely mixing together in water, and at room temperature, the clay, the zein and the zein dispersing agent; the operation requiring only from about one-half hour to one hour depending on the character of the ingredients. One may also prepare the zein-clay compound by separately dissolving the zein in a mixture of water and dispersing agent and then combining the zein solution or dispersion with the clay properly dispersed in

water. To prepare a casein-clay paper coating compound, the casein must be soaked in water for two to three hours and then dissolved with an alkali, or alkaline salt, soda ash, for example, at an elevated temperature, for instance at about 150° F., otherwise the coating material will be non-uniform and lumpy so as to interfere with proper printing.

(2) The amount of zein required to fix a given quantity of clay is less than the amount of casein required. For example, for ordinary printing paper about 10 to 12 parts of casein per 100 parts of clay, by weight, is required to give adequate adhesion. Equivalent results are obtained with 5 to 8 parts of zein. For higher gloss papers (referring to the gloss of the paper before printing) larger amounts of clay will be required and proportionately larger amounts of the protein binder. Under these circumstances the advantage of using zein in place of casein is enhanced.

(3) For gloss printing where a high gloss or varnish-like printed surface is required, it is ordinarily necessary to use between 16 and 20 parts of casein per 100 parts of clay. Equivalent 25 results in respect to the gloss of the printed surface may be obtained by using 10 to 12 parts of zein per 100 parts of clay.

It will be understood that the comparative figures given in the preceding numbered paragraphs 30 are approximate and typical. They are not intended to be exact for all operations.

(4) There is a special advantage in the use of a zein-clay coating for paper to be used for half-tone printing. The printing ink used for 35 the half-tone background consists of a dispersion of pigment in oil; and the background consists of scattered ink dots on the spots where the oily ink is able to overcome the oil resistance of the protein. Both casein and zein are oil resistant to a greater or less extent. Therefore, the smaller the ratio of protein to clay, the better will be the uniformity of the half-tone background. Where the protein content of the clay coating is high, the ink dots are larger and less uniform than when the protein content is lower. Moreover, it frequently happens that a small protein surface is so ink resistant that it does not take the ink at all and white spots result. This brings about an accumulation of unused ink on 40 the printing plate, producing, at the next paper contact, a larger ink spot than was intended. By reducing the ratio of protein to clay, as may be done with the substitution of zein for casein, the uniformity of the half-tone background is 45 much improved.

(5) A coating compound containing a given amount of casein will have a higher viscosity than one containing an equal quantity of zein. This difference is of considerable importance, particularly in the application of the coating to paper by means of a roll coating machine. With casein, in order to obtain the proper viscosity for the roll coating machine, it is necessary to dilute the casein-clay dispersion-suspension to about 35% solids and 65% water. At this dilution the coating compound deposits only a thin coating on the paper, for example, about 6 pounds of the coating per ream of paper. Therefore, in the case of roll coating machine operations, it has usually been found necessary, where the binder consists of casein, to give the paper two coatings in order that the necessary amount, say 12 pounds, of clay coating per ream may be deposited on the paper. Because of the lower viscosity of zein-clay dispersions of the same dry substance protein content, it is possible to increase the dry substance protein in the zein-clay coating compound and yet have the viscosity sufficiently low so as to make the compound workable on the roll coating machine. For example, experience has proven that zein-clay dispersions containing about 60% of solids and 40% of water may be used on the roll coating machine to deposit, in a single coating, about 12 pounds of clay coating per ream of paper.

(6) The cost of drying a zein-clay coating is less than the cost of drying a casein-clay coating. This appears to be due to two factors: lower viscosity, which makes possible higher concentration in the case of zein-clay coating compounds, so that there is less water to be dried out; and the fact that in the casein-clay compound the water is more closely held than in the zein-clay compound so that the moisture is less easily driven off.

For example, when the casein-clay coated paper is dried in a festoon drier of ordinary length, it may require a drying temperature between 120° and 130° F. With the zein-clay coating compound it has been found possible to do away entirely with artificial heating of the air. Or instead of this, the length of the drier, which is ordinarily very considerable, may be considerably reduced. Or the movement of the paper through the drier may be speeded up. In any case, the drying cost of the zein-clay coating is considerably reduced through increased capacity of the drying apparatus per unit of time or length of the drier, or through a reduction of temperature, or elimination of the heating apparatus and of temperature and humidity controls.

(7) The cost of the operation of the calender rolls, in the case of zein-clay coatings, is reduced. Zein has the property of producing a better gloss than casein when mixed with clay or its equivalent. For casein-clay coatings it is ordinarily necessary, if fairly high gloss is to be obtained, to weight the calender rolls in order to produce sufficient pressure to give the desired smoothness and gloss to the paper. It has been demonstrated that with zein-clay coated paper the calender rolls need not ordinarily be weighted at all, or the weights may be lighter, and this results in a saving of power.

(8) Another advantage follows from the thermoplasticity of zein. Casein containing coatings are substantially non-thermoplastic, that is, they retain their original rigidity when heated. Zein, on the contrary, becomes flexible under heat, or in other words, is thermoplastic. This

advantage of zein resulting from its thermoplasticity is particularly important where a zein-clay coated paper is used for embossing. In the embossing of clay coated paper the paper is subjected to an embossing roll, which roll, by pressure and friction, heats the coating. A zein-clay coating, because of its thermoplasticity, can be given the embossed design without substantial distortion of the paper itself. That is, the design can be raised on the coated side of the paper without correspondingly recessing or indenting the reverse side of the paper. This is not possible with a casein-clay coating.

15 The coating compound of the present invention consists essentially of a dispersion, preferably a water dispersion, of zein in which the zein is dispersed or dissolved by means of a suitable dispersing agent or agents, and clay or other filling substance carried in suspension in said zein dispersion.

20 Foam inhibitors are commonly used in connection with casein-clay coating compounds, and may be desirable in some instances in the case of the zein-clay compounds of the present invention. Suitable foam inhibiting substances are: pine oil; mixtures of pine oil and octyl alcohol; butyl alcohol; butyl stearate; amyl alcohol; lecithin; kerosene; and alum.

25 When certain zein dispersing agents are used, in accordance with the present invention, the use of foam inhibitors is not required or at least their use minimized, as will be hereinafter described.

30 The zein dispersing agent may consist of, or contain the following substances: rosin size, for example the sodium soap of rosin containing, for instance about 60% dry substance and 40% water, or other soaps of abietic acid containing substances such as the potassium, ammonium or 35 amine soaps of common rosins, hydrogenated rosins and ester gums; the sulfonated vegetable oils of the common vegetable oils, such as the castor oil; the soap of tall oil, which oil is a fatty acid mixture, that is the by-product of the wood pulp industry; the sulfonated mineral oils and—a preferred dispersing agent, as will be hereinafter described—sulfonated tall oil. The soaps of abietic acid containing substances, the soaps of other oils such as tall oils, and the sulfonated oils may 40 be used either singly or together. In fact, any solvent or dispersant of zein, or solvent or dispersant mixture of zein, which will give a zein solution or dispersion of sufficient viscosity to hold the required amount of clay or other inert filling material in suspension, may be employed 45 in this connection; and the term "zein dispersing agent," as used herein, is intended to cover all such substances and compounds. One may, for example, employ in this connection any of the zein dispersing agents described in applicant's 50 copending application, Serial No. 349,288, filed August 1, 1940, for "Zein dispersions and process of making the same," or any of the zein dispersing agents disclosed in the pending application of Albert Luther James, Serial No. 351,274, filed 55 August 3, 1940, for "Zein dispersions and processes of making same."

60 However, the present specification will give certain preferred dispersing agents and the methods of compounding the same with the clay to form zein-clay dispersions suitable for carrying out the present invention by processes which have been found desirable and expedient.

65 When the primary dispersing agent is a sulfonated oil or is an oil soap, it is preferable, but

not essential, to include in the compound small amounts of alkali such as caustic soda, caustic potash, ammonium hydroxide, borax, or one of the amines. The purpose of the use of small quantities of alkaline substances in this connection is to aid the primary dispersing agent in bringing about a complete dispersion of the zein. In such case the alkali is not used as a primary dispersing agent. The amounts used are too small for this purpose. The alkali does not form a reaction product with the zein as in the case when zein, as has been customary, is dissolved in strong, highly caustic solutions.

It is also preferable to mix a small amount of caustic alkali with the clay to facilitate its dispersion. The amount used is preferably about 0.1% of the clay, dry substance basis.

It is advantageous but not essential to incorporate urea with the other substances constituting the dispersing agent. It has been found that the addition of urea to a zein-clay coating compound increases the solubility of the zein and gives a lower viscosity for the same dry substance content, and thereby improves workability in the coating machines. Finally, the urea prevents the precipitation of the zein in aqueous dispersions where dispersing agents are used of such character as to reduce hydrogen ion concentration. For example, some of the sulfonated castor oils produce zein dispersions having pH's between 7 and 8. At this pH range the zein has a tendency to precipitate. The presence of urea retards this tendency.

A zein-clay dispersion will dry more quickly than a casein-clay dispersion. This may constitute an advantage, as indicated above; but in some cases it may be a detriment. For example, in the application of clay coatings with a brush coating machine, it is essential that the zein-clay coating should not dry or set so rapidly that the oscillating flat brushes, which follow the revolving cylindrical brush, will give an uneven or scratched surface to the coated paper.

The penetrating power of the dissolved protein element of a zein-clay dispersion is greater than the penetrating power of the protein in a casein-clay dispersion. The degree of penetration will naturally depend upon the fibrous character of the paper. When zein penetrates into the paper, separation necessarily takes place between the dissolved zein and the clay which latter is not capable of penetrating the paper to the same extent. This may result in lack of adhesion of the clay.

The too rapid drying of the zein solution and the tendency of the dissolved zein to penetrate the paper excessively may be counteracted, in accordance with the present invention by the addition of agents which thicken the dispersion and which may be designated as "drying and penetration retarding agents." These agents are all, generally speaking, of a colloidal or mucilaginous character, such as thick boiling starch pastes, that is, ordinary commercial, non-modified corn or other starches in a pasted condition; acid hydrolyzed, thin boiling starches; heat gelatinized or cold water swelling starches; thin boiling gelatinized or cold water swelling starches; viscous chlorinated starches; oxidized, thin boiling starches; and non-starch substances such as animal glue, soya bean protein, blood albumin, algin, casein, and methylcellulose.

For the purpose of retarding drying and penetration, the starch products are preferred; and experience with the several starch products, re-

ferred to above, indicate that a heat gelatinized or cold swelling tapioca starch gives the best results. In comparison with the other starch products referred to a lesser quantity is required to give the same viscosity; it has greater capacity for retarding the drying of the zein-clay coating. It assists in giving a better bond of the clay to the paper; it produces a finer colloidal dispersion and, for that reason, is able to retard the penetration of the zein into the interior of the paper sheet; and, being a cold water swelling or pasting product, it does not require cooking in order to paste it. However, any thickening colloidal or mucilaginous material can be used and will be effective to a certain extent. In general, one should use only the amount of starch or other agent which will retard drying and retard zein penetration to the desired extent without giving the zein-clay dispersion too high a viscosity for working conditions.

The use of starch in a zein-clay dispersion also appears to give a smoother surface to the finished coating.

The following are specific examples illustrating 25 the reduction of the present invention to practice. It will be understood, however, that these examples are purely illustrative and typical and are not to be considered as limiting the invention to the particular data given therein. The intention is to cover all equivalents and also all modifications within the scope of the hereto appended claims.

*Example 1.*—This compound is intended particularly for the roll type of coating machine. The compound consists of the following substances in quantities, by weight, as follows. (In all examples the quantities are by weight unless otherwise specified):

|                | Parts |
|----------------|-------|
| 40 Zein        | 100   |
| 60% rosin size | 170   |
| Water          | 1,115 |
| China clay     | 1,400 |

The rosin size consists of 60% dry substance 45 sodium rosin soap and 40% water. The dry substance in the rosin size may vary between 10% and 100%. The ratio of zein to rosin size, dry substance basis, may vary between 1 to 1 and 10 to 4.

The above ingredients are mixed together, at 50 room temperature, until the rosin soap has completely dissolved or dispersed the zein and until the clay has been uniformly suspended in the zein dispersion.

The compound in the specific proportions of 55 its ingredients given above contains about 60% of dry substance. The dry substance percentage may vary between 20% and 65%. The zein to clay ratio may vary between 5 to 100 and 12 to 60 100. The above noted possible variations indicate practical working ranges and not critical ranges. Generally speaking, the proportions between the ingredients will depend upon the character of the desired coating in respect to adhesiveness, 65 gloss of coating and gloss of the printed surface. In any case, the amount of rosin size must be sufficient to disperse the zein.

The product composed of the ingredients in 70 the proportions given above, specifically, will have the right consistency for use in connection with a roll coating machine.

The paper after being coated is passed through a festoon or other drier which need not be heated, although the use of heat is not excluded. The 75 coated paper may also be passed over heated

drums, or it may be dried by a combination of heated drums and festoon driers, or through a heated tunnel where the paper, suitably suspended or supported is subjected to a blast of air. Or the drying may be accomplished by any combination of heated drums, heated tunnels and festoon driers. In any case the drying will not require as much heat as in the case of casein-clay coated papers. The dried paper is then passed between the rolls of a series of pairs of 10 calendar rolls, which rolls, however, need not be weighted, or at least may have lighter weights than have been used heretofore.

The bond of this coating will be very strong, but the coating compound may have a tendency to foam so as to make advisable the use of foam inhibitors as described above.

*Example 2.*—This compound is intended particularly for use in connection with a brush coating machine. It consists of the following substances in quantities, by weight, as follows, possible variations being indicated in parentheses:

|                       | Parts            |
|-----------------------|------------------|
| Zein                  | 10 (6 to 12)     |
| Sulfonated castor oil | 4 (1 to 12)      |
| Caustic soda          | 0.4 (0.2 to 0.6) |
| Water                 | 125 (80 to 150)  |
| China clay            | 100              |

This formula, with the ingredients in the preferred proportions indicated above, gives a zein-clay compound containing 45% dry substance, whereby the material has a sufficiently fluid consistency to make it applicable to the paper by means of a brush machine. The other steps of the process may be the same as given in Example 1.

It will be understood, in connection with this and other formulas giving quantity ranges, that, generally speaking, a change in the quantity of one ingredient from the specified preferred amount should be accompanied by a corresponding change in the quantities of the other ingredients in order to obtain the best results.

*Example 3.*—The coating compound consists of the following substances in quantities, by weight as follows:

|                                  | Parts          |
|----------------------------------|----------------|
| Zein                             | 8 (6 to 12)    |
| 85% sulfonated castor oil        | 3 (3 to 5)     |
| Ammonium rosin (Staybelite size) | 5 (3 to 8)     |
| Water                            | 90 (85 to 150) |
| China clay                       | 100            |

By "85% sulfonated castor oil" is intended a sulfonated castor oil having a water content of about 15%.

Approximately one-third of the water (not counting that in the sulfonated castor oil) is mixed with the sulfonated castor oil and the ammonium rosin size, and the zein dispersed in this mixture. Into the zein dispersion, thus formed, is mixed the clay and the rest of the water, and the mixture is puddled until all lumps are removed.

The above described clay coating compound may be used either on a roll or brush coating machine, after proper adjustment of viscosity and dry substance content. The resulting coating has been found to be superior in respect to water resistance and color to the coatings produced in accordance with Examples 1 and 2. It is believed that the ammonium rosin size contributes to improved color and improved water resistance.

Staybelite, being a hydrogenated rosin, is considerably lighter in color than ordinary rosin.

*Example 4.*—If still better color is desired this can be obtained by dissolving the rosin of Example 3 in the minimum quantity of ethyl alcohol or isopropyl alcohol required to dissolve it before combining the rosin with the ammonia to produce the soap. The alcohol also promotes the more rapid solution of the zein and acts to minimize foaming.

*Example 5.*—The compound consists of the following ingredients, by weight, as follows (the figures in parentheses indicating practical not critical ranges):

|                           | Parts            |
|---------------------------|------------------|
| Zein                      | 8 (6 to 12)      |
| 85% sulfonated castor oil | 3 (2 to 8)       |
| Sodium aluminate          | 0.4 (0.3 to 1.0) |
| Urea                      | 4 (1 to 8)       |
| Water                     | 85 (80 to 100)   |
| China clay                | 100              |

The zein is dispersed in the sulfonated castor oil and 25 parts (20 to 40 parts) of the water, and to this is added the mixture of urea and sodium aluminate. The clay is puddled with the rest of the water until all lumps are removed and the zein dispersion is then mixed with the clay suspension. With the preferred amounts indicated above, this will give a clay coating compound containing about 57.5% dry substance.

*Example 6.*—The coating compound consists of the following ingredients in quantities, by weight, as follows:

|                           | Parts          |
|---------------------------|----------------|
| Zein                      | 8 (6 to 12)    |
| 85% sulfonated castor oil | 4 (3 to 8)     |
| Urea                      | 4 (3 to 8)     |
| Water                     | 85 (80 to 100) |
| China clay                | 100            |

It will be noted that in this example the alkaline sodium aluminate of Example 4 is omitted.

*Example 7.*—The coating compound consists of the following substances in quantities, by weight, as follows:

|                           | Parts          |
|---------------------------|----------------|
| Zein                      | 8 (6 to 12)    |
| 85% sulfonated castor oil | 3 (2 to 8)     |
| Borax                     | 1 (0.8 to 2)   |
| Urea                      | 4 (1 to 8)     |
| Water                     | 85 (80 to 100) |
| China clay                | 100            |

*Example 8.*—The compound consists of the following substances in quantities, by weight, as follows:

|                                                             | Parts          |
|-------------------------------------------------------------|----------------|
| Zein                                                        | 8 (6 to 12)    |
| 85% sulfonated castor oil                                   | 3 (2 to 8)     |
| Concentrated ammonium hydroxide solution, 28% concentration | 1              |
| Urea                                                        | 4 (1 to 8)     |
| Water                                                       | 85 (80 to 100) |
| China clay                                                  | 100            |

*Example 9.*—The compound consists of the following substances in quantities, by weight, as follows:

|                           | Parts          |
|---------------------------|----------------|
| Zein                      | 8 (6 to 12)    |
| 85% sulfonated castor oil | 3 (2 to 8)     |
| Triethanolamine           | 3              |
| Urea                      | 4 (1 to 8)     |
| Water                     | 85 (80 to 100) |
| China clay                | 100            |

*Example 10.*—The compound consists of the following substances in quantities, by weight, as follows:

|                           | Parts          |
|---------------------------|----------------|
| Zein                      | 8 (6 to 12)    |
| 85% sulfonated castor oil | 3 (2 to 8)     |
| Trisodium phosphate       | 0.5            |
| Urea                      | 4 (1 to 8)     |
| Water                     | 85 (80 to 100) |
| China clay                | 100            |

*Example 11.*—The compound consists of the following substances in quantities, by weight, as follows:

|                                 | Parts          |
|---------------------------------|----------------|
| Zein                            | 8 (6 to 12)    |
| Sulfonated mineral oil          | 4 (2 to 8)     |
| Concentrated ammonium hydroxide | 2 (1 to 3)     |
| Urea                            | 4 (1 to 8)     |
| Water                           | 85 (80 to 100) |
| China clay                      | 100            |

*Example 12.*—The compound consists of the following substances in quantities, by weight, as follows:

|                                 | Parts          |
|---------------------------------|----------------|
| Zein                            | 8 (6 to 12)    |
| Sulfonated mineral oil          | 4 (3 to 6)     |
| Concentrated ammonium hydroxide | 2 (1.5 to 3)   |
| Urea                            | 4 (1 to 8)     |
| Water                           | 85 (80 to 100) |
| China clay                      | 100            |

*Example 13.*—The compound consists of the following substances in quantities, by weight, as follows:

|                           | Parts          |
|---------------------------|----------------|
| Zein                      | 8 (6 to 12)    |
| 85% sulfonated castor oil | 3 (2 to 8)     |
| Sodium aluminate          | 0.4 (0.3 to 1) |
| Urea                      | 4 (1 to 8)     |
| Water                     | 85 (80 to 100) |
| China clay                | 100            |
| Algin                     | 0.4 (0 to 1)   |

Algin, used herein as a drying and penetration retarding agent, is a by-product obtained during the extraction of iodine from sea kelp.

*Example 14.*—The coating compound consists of the following substances in quantities, by weight, as follows:

|                                              | Parts          |
|----------------------------------------------|----------------|
| Zein                                         | 8 (6 to 12)    |
| 85% sulfonated castor oil                    | 3 (2 to 8)     |
| Borax                                        | 1 (1 to 2)     |
| Urea                                         | 4 (1 to 8)     |
| Water                                        | 85 (80 to 100) |
| China clay                                   | 100            |
| Sodium peroxide modified thin boiling starch | 2.5            |

The sodium peroxide modified thin boiling starch, which may have a fluidity of about 80, is used as a drying and penetration retarding agent. The oxidized starch should be added in the pasted state. This is preferably accomplished by cooking the 2.5 parts of starch with 6 parts of water. Other oxidized starches might be used.

*Example 15.*—The compound consists of the following substances in quantities, by weight, as follows:

|                                                  | Parts      |
|--------------------------------------------------|------------|
| Zein                                             | 8          |
| 85% sulfonated castor oil                        | 3          |
| Water                                            | 100        |
| China clay                                       | 100        |
| Heat gelatinized or cold swelling tapioca starch | 3 (3 to 5) |

The gelatinized tapioca starch is dissolved in 40 parts of the water, which may be cold. The china clay mixed with the rest of the water is added to the starch suspension. Finally, the zein-sulfonated castor oil-caustic soda mixture is mixed thoroughly with the clay-starch suspension. It appears to be desirable, if not necessary, to add the starch to the clay mix before compounding with the zein mix in order to obtain a smooth, non-lumpy and uniform mixture of all ingredients.

*Example 16.*—The compound consists of the following substances in quantities, by weight, as follows:

|                                 | Parts |
|---------------------------------|-------|
| Zein                            | 6     |
| 85% sulfonated castor oil       | 3     |
| Sodium aluminate                | 0.3   |
| Water                           | 100   |
| China clay                      | 100   |
| Thin boiling chlorinated starch | 6     |

A paste is made by cooking the thin boiling chlorinated starch in 40 parts of the water. The clay is puddled in the rest of the water. The paste is cooled and all of the ingredients mixed together, namely: the clay-water dispersion, the zein-sulfonated oil dispersion, and the cold starch paste.

*Example 17.*—The formula here is the same as in Example 16 except that animal glue is used in place of starch paste. 2 parts of animal glue are mixed with 4 parts of the specified amount of water and heated to a paste. 10 parts more of the water is added to the paste and the ingredients mixed as in Example 16.

*Example 18.*—The compound consists of the following substances in quantities, by weight, as follows:

|                                  | Parts |
|----------------------------------|-------|
| Zein                             | 10    |
| 85% sulfonated castor oil        | 3.75  |
| 1/2 normal caustic soda solution | 8.5   |
| Water                            | 100   |
| China clay                       | 100   |
| Methylcellulose                  | 1     |

The methylcellulose acts as a drying and penetration retarder.

The zein, sulfonated castor oil, caustic soda solution and 27.5% of the water are mixed together to form a zein dispersion. The clay, the rest of the water and the methylcellulose are mixed together and the two mixtures combined.

*Example 19.*—The compound consists of the following substances in quantities, by weight, as follows:

|                    | Parts          |
|--------------------|----------------|
| Zein               | 8 (6 to 16)    |
| Tall oil           | 4 (4 to 12)    |
| Urea               | 4 (2 to 8)     |
| Ammonium hydroxide | 2 (2 to 6)     |
| Water              | 85 (60 to 200) |
| China clay         | 100            |

*Example 20.*—The compound consists of the following substances in quantities, by weight, as follows:

|                         | Parts            |
|-------------------------|------------------|
| Zein                    | 8 (6 to 16)      |
| 63% sulfonated tall oil | 5 (2 to 8)       |
| Caustic soda            | 0.4 (0.3 to 0.5) |
| Water                   | 100 (60 to 200)  |
| China clay              | 100              |

63% sulfonated tall oil has a water content of 37% not included in the specified 100 parts.

0.3 part of the caustic soda is used in making the zein-sulfonated tall oil dispersion. 0.1 part of the caustic soda is used in puddling the clay and the rest of the water in order to obtain a better dispersion of the clay.

This expedient of using a small amount of an alkaline substance, particularly a caustic alkali, to improve the dispersion of the clay in the water, may be employed in any of the examples given above.

The zein-clay coating compound of this example has certain definite advantages as follows: (a) The zein is dispersed more quickly. With most of the zein dispersions made from sulfonated castor oil or rosin size, it is necessary to mix the ingredients for about an hour, whereas, by the use of this formula the dispersion may be effected in about 30 minutes. (b) The use of sulfonated tall oil results in almost complete elimination of foaming difficulties. (c) The finished coating is lighter in color. (d) A zein-clay dispersion in accordance with this example has viscosity and body enough for use in connection with a roll coating machine and, at the same time, is fluid enough for use with a brush coating machine. (e) Printing characteristics are improved because of more uniform absorption of the printing ink.

*Example 21.*—The compound consists of the following substances in quantities, by weight, as follows:

|                                                                 | Parts             |
|-----------------------------------------------------------------|-------------------|
| Zein                                                            | 16 (12 to 32)     |
| 63% sulfonated tall oil                                         | 5 (4 to 12)       |
| Potassium rosin size made from hydrogenated rosin (Staybel-ite) | 10 (4 to 20)      |
| Sodium hydroxide                                                | 0.4 (0.3 to 0.75) |
| Water                                                           | 200 (150 to 400)  |
| China clay                                                      | 200               |
| Heat gelatinized tapioca starch                                 | 6 (2 to 10)       |

The sodium hydroxide is dissolved in 2.5 parts of the water and the gelatinized tapioca starch in the rest of the water. The china clay is mixed with the water mixture of the starch and this mixture is combined with the zein, sulfonated tall oil, rosin and sodium hydroxide dispersion. About 0.1 part of the caustic soda is introduced into the clay suspension before this suspension is added to the zein dispersion.

In both Examples 20 and 21 in which sulfonated tall oil is used, it appears to be important, if the best results are to be obtained, to introduce into the compound a small quantity of an alkaline substance, particularly caustic soda or caustic potash. It also appears to be important to introduce into the clay a small quantity of the caustic when the clay is puddled with the water or diluted starch paste.

In place of the zein dispersing agents mentioned in the foregoing examples one may use any of the zein dispersing agents disclosed in the application of Stewart, Serial No. 349,288, which,

in all cases, involve a certain amount of alcohol, aqueous ethyl, methyl, isopropyl, or high boiling point organic zein solvent, but with water also present in such large quantity that, except for the dispersing agent, the zein would be precipitated. As set forth in the Stewart application, dispersing agents suitable for the purposes of the present invention include the following water soluble, highly ionized, compounds containing 8 or more carbon atoms: (1) the alkali metal, ammonia and amine soaps; (2) the sulfonated vegetable oils; (3) the sulfated and sulfonated fatty acids and alkali metal, ammonia and amine and other water soluble salts of said sulfated and sulfonated fatty acids; (4) the sulfated and sulfonated fatty alcohols and the alkali metal, ammonia, amine and other water soluble salts of said sulfated and sulfonated fatty alcohols; (5) the alkali metal, ammonia, amine and other water soluble salts of alkyl, aryl, alkyl aryl, and heterocyclic sulfonic acids; (6) the salts of aryl carboxylic acid; and (7) derivatives of any of these groups which contain at least eight carbon atoms in the organic radical and substituent group taken together.

As specific examples of the groups just mentioned one may employ the following: rosin soap formed by combining rosin with caustic soda; amine laurate soap formed by combining lauric acid with triethanolamine; amine soap formed by combining lauric acid with monomethylamine; ammonium soap of rosin; ammonium soap of linseed oil fatty acids; rosin soap composed of rosin and morpholine; sodium stearate; sulfated stearyl alcohol (Avitex S. F.); sodium salt of alkyl naphthalene sulfonic acid (Nekal B. X.); oleyl ethane sulfonic acid salt derived by extraction with alcohol from the commercial product Igepon A. P.

One may also use any of the zein dispersing agents disclosed in said application of Albert Luther James, Serial No. 251,274, in which alcohol is preferably absent, as follows: (1) the alkali metal, ammonia, and amine soaps; (2) the sulfonated vegetable oils; (3) the sulfated and sulfonated fatty acids and the alkali metal, ammonia, amine and other water soluble salts of said sulfated and sulfonated fatty acids; (4) the sulfated and sulfonated fatty alcohols and the alkali metal, ammonia, amine and other water soluble salts of said sulfated and sulfonated fatty alcohols; (5) the alkali metal, ammonia, amine, and other water soluble salts of the alkyl, aryl, alkyl aryl, and heterocyclic sulfonic acids; (6) the salts of aryl carboxylic acid; and (7) derivatives of any of these groups which contain at least eight carbon atoms in the organic radical and substituent group taken together.

As specific examples of the groups just mentioned are the following: the reaction product of sulfonated linseed or soyabean oil with ammonium hydroxide; the sulfated fatty alcohols or their alkali, ammonia or amine salts, such for example as sodium lauryl sulfate (Duponol M. E.); ammonium stearate, or any water soluble salt of a fatty acid containing over twelve carbon atoms, for example sodium oleate or potassium palmitate; the mixture of sulfonated castor oil, tall oil and ammonium hydroxide; sodium laurate; ammonium soap of linseed fatty acids; triethanolamine oleate; triethanolamine palmitate; ammonium naphthenate; sodium soap produced by the reaction of stearic acid with sodium hydroxide; Avitex S. F.; Nekal B. X.; Triton

1-18, a reaction product of a fatty acid with an aryl alkylated amine; Decersol O. T., a sodium salt of a sulfate of dicarboxylic acid ester; Igepon A. P.

I claim:

Composition of matter suitable for coating paper comprising the following substances in quantities, by weight, substantially as follows:

zein 12 to 32 parts; sulfonated tall oil 4 to 12 parts; potassium rosin size made from hydrogenated rosin 4 to 20 parts; sodium hydroxide 0.3 to 0.75 part; water 150 to 400 parts; china clay 200 parts; heat gelatinized tapioca starch 2 to 10 parts.

CHARLES W. STEWART.